

Jan. 1, 1952

N. E. WIDELL

2,580,983

CORROSION INHIBITORS IN ABSORPTION REFRIGERATION SYSTEM

Filed Feb. 8, 1946



INVENTOR.

*Nils Erik Widell*  
BY

*D. E. Hatch  
his Attorney*

## UNITED STATES PATENT OFFICE

2,580,983

CORROSION INHIBITORS IN ABSORPTION  
REFRIGERATION SYSTEMNils Erik Widell, Stockholm, Sweden, assignor to  
Aktiebolaget Electrolux, Stockholm, Sweden, a  
corporation of SwedenApplication February 8, 1946, Serial No. 646,394  
In Sweden January 22, 1945

15 Claims. (Cl. 62—179)

**1** This invention relates to absorption refrigerating apparatus and more particularly to such apparatus of the inert gas type wherein the absorption solution contains a corrosion protective substance. The main object of the invention is to increase the lifetime of the apparatus and to prolong the durability of the corrosion protection. The invention is of particular importance in such refrigerating apparatus wherein absorption solution from its normal circulating system through the boiler and absorber of the apparatus is brought into contact with working medium having a higher refrigerant concentration than that of the absorption solution.

The invention will be hereinafter more fully described with reference to the accompanying drawing showing diagrammatically an embodiment of the arrangement according to same and in this connection further characteristic features of the invention will be set forth.

The figure shows diagrammatically an absorption refrigerating apparatus, wherein water is used as an absorbent and ammonia as refrigerant. Referring to the figure reference numeral 10 denotes a tube acting as a flue, to which heat is continuously supplied from a heat source, not shown, for example an electric cartridge, a gas or petroleum burner. The boiler of the apparatus is designated by 11 and its liquid circulating pump by 12. The boiler pipe 11 is extended upwardly and at the top connected to the air cooled condenser 13 of the apparatus. Further numeral 14 denotes a so-called pressure equalizing vessel of a kind known per se which through a drainage conduit 15 communicates with the evaporator of the apparatus designated by 16. In said conduit 15 the condenser pipe 13 opens, from which liquid refrigerant thus flows by gravity to the evaporator through the conduit 15. Further numeral 17 designates the gas heat exchanger of the apparatus and 18 its air-cooled absorber. Numeral 19 indicates a vent conduit through which the pressure equalizing vessel 14 freely communicates with the gas circulating system of the apparatus. Said system is formed in a way known per se as is the liquid circulating system of the apparatus. The enriched solution in the absorber vessel 20 of the apparatus thus streams through its liquid heat exchanger 21 and the main pump 12 to the boiler 11 and thence it returns through the heat exchanger 21 and a conduit 22 to the absorber 18.

In accordance with usual practice the apparatus is formed of iron pipes joined together by gas welding. Before filling the apparatus it is

**2** evacuated of all air, and as ammonia by itself has no influence upon iron in absence of oxygen, no corrosion should be feared in the internal iron walls. However, these walls formed of ferrous metal will nevertheless be affected by the ammonia solution by the forming of complicated iron compounds, by which the walls after a relatively short time would be loosened up and lose their strength against the high pressure (about 20 atm.) prevailing in the apparatus. In order to avoid such corrosion an alkali salt of sodium chromate ( $Na_2CrO_4$ ) has previously been dissolved in the absorption solution. The chromatic concentration required in the absorption solution for counteracting the corrosion is extremely small and may be counted in fractions of per cent. However, the chromate is slowly consumed and therefore it has previously been necessary to utilize a concentration of chromate in the solution many times higher for the purpose of creating a chromatic reserve, covering several years' consumption. Salts dissolved in the absorption solution will, however, influence the pumping in the thermosiphon pump 12 in a unfavourable direction and therefore until now it has been necessary to limit the concentration of chromate in the solution to a concentration corresponding to about 2% of  $CrO_3$ .

In different ways, however, it has been attempted to form an additional reserve of alkali chromate by enclosing in the absorber vessel a storage of solid sodium chromate in a container with a limited communication with the surrounding solution, whereby a gradual dissolving of the solid chromate has been attained. It has not been possible to make the dissolving so uniform that the concentration of the solution with security can be kept below the values wanted. The velocity of dissolving has also appeared to be dependent upon a plurality of uncontrollable factors, among other things the operating temperature which very essentially varies with the climatic concentration under which the apparatus is operated. According to this invention a reserve of chromate of an arbitrary greatness may be arranged in the apparatus. The invention is substantially characterized thereby that the absorption solution of the apparatus is saturated with a salt of the chromatic acid, having a solubility in said solution not exceeding 2%. Further the solubility of the present chromate may be as much as possible independent of the temperature, though certain variations with the temperature may be permitted. A particularly suitable chromate is strontium chromate ( $SrCrO_4$ ). The solu-

bility of strontium chromate in the absorption solution is so small that the saturated solution only contains 0.01 to 0.2% of  $\text{CrO}_3$ .

Apparently this small quantity of chromate which originally, when filling the apparatus, is dissolved in the absorption solution will be comparatively rapidly consumed. It is therefore generally necessary to enclose a reserve of solid strontium chromate in the apparatus. According to the invention therefore a container 50 is arranged in the absorber vessel 20 or possibly in another vessel interconnected with the liquid circulating system of the apparatus. The reservoir 50 may suitably include a short piece of pipe, both openings of which are covered with a fine-meshed iron net and in which a pressed tablet of strontium chromate is inserted. The container may suitably be attached to the wall of the vessel by a strip or similar member which is attached to the wall of the vessel and to the wall of the container 50 by welding. The support is denoted by 51. When the liquid contents of the absorber vessel 20 is continuously renewed, the absorption solution will automatically become saturated gradually as its contents of chromate decreases during its passage through the absorber vessel 20. The pressing of the solid strontium chromate into a tablet possesses the advantage that no solid particles by mechanical influence of the streaming solution will follow the liquid through the narrow passages of the apparatus. In order to improve the strength of the tablet small amounts of sodium hydroxide may be mixed with the chromate when pressing said tablet.

As already mentioned, the invention is of particular importance in such absorption refrigerating apparatus in which the absorption solution is now and then brought into contact with liquid refrigerant, the concentration of which thus attains high values. This is the case in the absorption refrigerating apparatus shown in the figure. From the lower part of the boiler pipe a conduit 23 runs out, which opens into the pressure equalizing vessel 14 and forms an auxiliary pump for raising the absorption solution to said vessel. Thence, the warm solution streams through the conduit 15 into the evaporator coil 16 and thence through the exchanger 17 and the absorber 18 to the absorber vessel 20. In contradistinction to the main pump 12 the auxiliary pump 23 is not immediately heat conductively connected with the flue 10 but instead arranged in heat conductive relation with a hermetically closed heat transfer system which is welded to the flue 10 along a welded seam 42. The system contains a heat transfer medium with a high boiling point, possibly in addition to an auxiliary medium with a lower boiling point. The transfer medium is vaporized in the boiling part 41 of the system and condenses to liquid in a container 30 where the condensate is accumulated. Some part of the vapours, however, give off their heat contents to the pump pipe 23. After a certain period the system is boiled dry, and all the condensate remains stored in the container 30. This container is connected by a flexible member 31 with the system, thus permitting it to be raised for tilting the liquid contents. In this way a method of controlling the heat transfer system is attained, thus causing the pump 23 to operate whenever desired and after a certain period automatically to stop working. The solution raised by the auxiliary pump 23 streams in the way already described into the evaporator where it, however, is mixed with refrigerant condensate

entering from the condenser 13, having an ammonia concentration from 80 to 100%. The supply of condensate from the condenser 13 takes place continuously. This supply of absorption solution to the evaporator 16 has for its object, when required, to effect melting of ice formed thereon. It has appeared that a solution of sodium chromate of 1 to 2 per cent cannot be mixed with ammonia having the concentration existing in the evaporator without most of the salt being precipitated into solid form. The salt precipitated would collect in the evaporator and would very soon effect a blocking action and at the same time such precipitated salt for the future would be prevented from taking part of the corrosion protection. A solution of strontium chromate remains, even if it is saturated, approximately unaffected by an increase of the ammonia concentration and the small amounts of chromate which possibly may be precipitated will be replaced from the reserve 50 provided in the absorber vessel.

Though the strontium chromate is very little soluble in the absorption solution, that is, in the ammonia water mixture, the concentration of protecting substance in this chemical compound is sufficient to effect a satisfying corrosion protection. Other chromates, such as lead chromate, neutral or basic ( $\text{PbCrO}_4$  or  $\text{PbCrO}_4 \cdot \text{PbO}$ ) are practically insoluble in the ammonia water solution. Accordingly such compounds alone and by themselves have no corrosion protective effect. According to the invention, however, the active substance of the lead chromate may be freed from the lead when in the absorption solution an activating substance is dissolved, such as sodium hydroxide ( $\text{NaOH}$ ) or any other substance which when disintegrated forms sodium hydroxide. According to another phase of the invention, sodium hydroxide, for example 2%, is dissolved in the absorption solution. This solution will then effect a disintegration of the lead chromate, substantially according to the following form:



The sodium chromate formed thereby will be dissolved by the absorption solution and distributed into all parts of the circulation system of the absorption solution. The lead compound  $\text{NaHPbO}_2$  is also soluble in the absorption solution, and therefore will not effect any disturbances. According to the small concentration of the sodium hydroxide in the solution, the quantity of sodium chromate formed and dissolved therein in accordance with the foregoing equation will be small and will remain at a substantially constant value as the reaction proceeds until all lead chromate has been dissolved.

In some cases the low concentration of the chromate in the absorption solution will be insufficient for effecting a satisfactory protection against corrosion. According to a further phase of the invention, however, a further corrosion protective substance, such as the nitrites of alkali metals, for example, may be added to the absorption solution and dissolved therein until a concentration of about 4% is attained. Such nitrites of the alkali metals may include ammonium, potassium or sodium nitrite. Preferably sodium nitrite ( $\text{NaNO}_2$ ) is used. Though this chemical compound by itself is known as being very unstable investigations have shown that the duration of the protective effect is sufficient for the above purpose and may be very much increased when

a chromate, also a very diluted solution of chromates, is used in combination with the nitrites. The concentration of chromates sufficient for effecting such an increase of the duration of diluted nitrite solutions corresponds to about 0.02 to 0.2%  $\text{CrO}_3$ . It is evident that nitrite solutions containing 0.02 to 4%  $\text{NaNO}_2$  and saturated with strontium chromate or lead chromate is very suitable as absorption solutions in refrigerating apparatus of the above described type, due to the fact that sodium nitrite when acting as a corrosion protective substance will be disintegrated forming thereby gaseous products and sodium hydroxide. This sodium hydroxide will dissolve lead chromate as described above, and accordingly activate said compound which in itself is practically insoluble and inactive. The sodium hydroxide and the sodium nitrite respectively accordingly act as activators for the lead chromate. The sodium chromate dissolved thereby prevents the rapid disintegration of the nitrites.

It is evident that the invention is of greatest importance in connection with hermetically closed refrigerating apparatus of the type described in connection with the figure. The lifetime of such apparatus is substantially determined by the duration of the corrosion protection. According to the invention it is now possible to enclose in such apparatus a corrosion protective substance soluble in the absorbent and useable in high concentration, and a second corrosion protective substance acting as conservator for said first corrosion protective substance and a reserve of solid corrosion protective substance, from which an active part is dissolved by means of the disintegration products of the first-mentioned corrosion protective substance. Due to this fact the corrosion protection may be made effective for an extremely long duration.

I claim:

1. In the art of refrigeration employing an hermetically sealed absorption refrigerating system formed of ferrous metal and having an absorption solution circuit in which aqueous ammonia solution is circulated through and between a place at which ammonia is expelled from solution and a place at which ammonia is absorbed into solution, the improvement which comprises maintaining in the solution a supply of solid lead chromate, and providing in the solution an alkali nitrite.

2. The improvement as set forth in claim 1 in which sodium nitrite is provided in an amount to obtain a concentration of from 0.02 to 4.0 per cent.

3. In the art of refrigeration employing an hermetically sealed absorption refrigerating system formed of ferrous metal and having an absorption circuit in which an aqueous ammonia solution is circulated through and between a place at which ammonia is expelled from solution and a place at which ammonia is absorbed into solution, the improvement which comprises maintaining in the solution a supply of solid lead chromate, and making available in the solution an alkaline hydroxide.

4. The improvement as set forth in claim 3 in which about 2 per cent sodium hydroxide is added to the solution.

5. In the art of refrigeration employing an hermetically sealed absorption refrigerating system formed of ferrous metal and containing ammonia, water and hydrogen and comprising an evaporator and a number of parts interconnected to provide a circuit for circulation of aqueous ammo-

nia solution and in which such solution is supplied at will from said circuit to the evaporator to effect defrosting of the latter when desired, the improvement which comprises adding to the solution an alkaline nitrite, and maintaining in said circuit a supply of a chromate salt of lead which is in solid form.

6. The improvement as set forth in claim 5 in which sodium nitrite is added to the solution.

7. In the art of refrigeration employing an absorption refrigeration system formed of ferrous metal and utilizing ammonia as refrigerant and water as an absorbent, that improvement which comprises maintaining in the aqueous ammonia solution in physical contact therewith a supply of a chromate salt of lead soluble in the solution only with difficulty and having bound therein a chromate radical inactive due to the insolubility of said lead salt, and adding to the solution another substance which upon dissolution or disintegration will provide an alkaline hydroxide to effect liberation of said chromate radical by chemical action.

8. In the art of refrigeration employing an absorption refrigeration system formed of ferrous metal and utilizing ammonia as refrigerant and water as an absorbent, that improvement which comprises maintaining in the aqueous ammonia solution in physical contact therewith a supply of a chromate salt of lead soluble in the liquid only with difficulty and having bound therein an inactive chromate radical capable of forming a readily soluble corrosion inhibiting chromate salt upon liberation from said lead salt, and providing in the solution an alkali hydroxide which will effect liberation of said inactive chromate radical from said lead salt and promote formation of said corrosion inhibiting chromate salt.

9. In the art of refrigeration employing an absorption refrigeration system formed of ferrous metal and utilizing ammonia as refrigerant and water as an absorbent, that improvement which comprises maintaining in the aqueous ammonia solution in physical contact therewith a supply of a chromate salt of lead soluble in the solution only with difficulty and having bound therein a corrosion resisting chromate radical inactive due to the insolubility of said lead salt, and adding to the solution an alkali nitrate effective to inhibit corrosive action which upon disintegration thereof will liberate said corrosion resisting chromate radical by chemical action.

10. In the art of refrigeration employing an absorption refrigeration system formed of ferrous metal and utilizing ammonia as refrigerant and water as an absorbent, that improvement which comprises maintaining in the aqueous ammonia solution in physical contact therewith a supply of chromate salt of lead soluble in the solution only with difficulty and having chemically bound therein an inactive chromate radical capable of forming a readily soluble corrosion inhibiting chromate salt upon liberation from the said lead salt, adding to the solution an alkali nitrate which upon dissociation is effective to liberate said inactive chromate radical from the said lead salt to produce said readily soluble corrosion inhibiting chromate salt, and utilizing said readily soluble corrosion inhibiting chromate salt to retard and slow down rate of dissociation of said alkali nitrate.

11. In the art of refrigeration employing an absorption refrigeration system formed of fer-

7

rous metal and utilizing ammonia as refrigerant and water as an absorbent, that improvement which comprises maintaining in the aqueous ammonia solution in physical contact therewith a supply of solid lead chromate compound ( $PbCrO_4$  or  $PbCrO_4$ ,  $PbO$ ), said compound being soluble in the solution only with difficulty and thereby rendering the chromate inactive as a corrosion inhibiting agent, and liberating the chromate from said compound and forming a corrosion inhibiting chromate compound soluble in the solution by adding a substance selected from a group consisting of an alkali nitrite or an alkali hydroxide.

12. In the art of refrigeration employing an absorption refrigeration system formed of ferrous metal and utilizing ammonia as refrigerant and water as an absorbent, that improvement which comprises maintaining in the aqueous ammonia solution a solid substance comprising a chromate salt of lead, and adding an alkali nitrite to the solution. 15 20

13. In the art of refrigeration employing an absorption refrigeration system formed of ferrous metal and utilizing ammonia as refrigerant and water as an absorbent, that improvement which comprises maintaining in the aqueous ammonia solution a solid substance comprising a chromate salt of lead, and adding an alkali hydroxide to the solution.

14. The combination with an absorption refrigeration apparatus formed of ferrous metal which includes a number of parts interconnected to provide a circuit for active circulation of aqueous ammonia solution having a corrosion inhibiting chromate salt soluble therein, said parts including a boiler or generator and an

8

absorber comprising a looped coil and vessel connected thereto, means to provide said soluble corrosion inhibiting chromate salt including a tablet in solid form comprising a substance selected from a group consisting of strontium chromate ( $\text{SrCrO}_4$ ), neutral lead chromate ( $\text{PbCrO}_4$ ) or basic lead chromate ( $\text{PbCrO}_4$ ,  $\text{PbO}$ ), and means comprising a receptacle for holding said tablet in said vessel in intimate contact with the aqueous ammonia solution therein at a region removed from the walls defining said vessel.

15. In the art of refrigeration employing an absorption refrigeration system formed of ferrous metal and utilizing ammonia as refrigerant and water as an absorbent, that improvement which comprises providing in the system a soluble alkali nitrite and a solid substance selected from a group consisting of strontium chromate ( $\text{SrCrO}_4$ ), neutral lead chromate ( $\text{PbCrO}_4$ ) or basic lead chromate ( $\text{PbCrO}_4 \cdot \text{PbO}$ ).

NILS ERIK WIDELL.

#### REFERENCES CITED

The following references are of record in the  
25 file of this patent:

UNITED STATES PATENTS

| Number    | Name       | Date                       |
|-----------|------------|----------------------------|
| 1,960,040 | Widell     | May 22, 1934               |
| 2,210,611 | Widell     | Aug. 6, 1940               |
| 2,246,665 | Buffington | June 24, 1941              |
| 2,402,413 | Kogel      | June 1 <sup>o</sup> , 1946 |
| 2,457,334 | Widell     | Dec. 28, 1946              |

## FOREIGN PATENTS

Number 117,816 Country Australia Date Dec. 1943